

## UNITED STATES PATENT OFFICE

2,673,143

PRODUCING A MIRRORLIKE FINISH  
ON ALUMINUM

Eugene R. Du Fresne, Chicago, and John R. Swihart, Chicago Heights, Ill., assignors to The Diversey Corporation, a corporation of Illinois

No Drawing. Application March 10, 1951,  
Serial No. 215,031

15 Claims. (Cl. 41—42)

This invention relates to the production of a mirrored surface on aluminum, a bath for producing it, and the products so produced.

In the ordinary commercial production of aluminum, the material, after fabrication, is customarily etched to remove surface scratches and produce a satin finish. It has now been discovered that by using an etching bath composed of sodium gluconate, sodium hydroxide, and sodium nitrate, the resulting finish instead of being satin is a highly mirrored reflecting surface.

Acid baths for producing a mirrored surface have heretofore been suggested, but they are expensive, require special tanks, require high concentrations of acids, and there is considerable loss due to drag out.

The present invention utilizes caustic soda baths including an oxidizing agent and a water soluble saturated aliphatic polyhydroxy compound of the class consisting of sorbitol, gluconic acid its salts and lactones and mucic acid its salts and lactones.

Glycerine and gum arabic have been found desirable additives in that they keep the accumulation of smut at a minimum, and thus assist in the achievement of a better polish.

The preferred oxidizing agent is sodium nitrate. Sodium chlorate and sodium nitrite are also quite satisfactory. Sodium perchlorate and sodium hypochlorite are less satisfactory, but have some polishing effects. A combination of sodium nitrate and sodium chlorite gave very good results with considerably less total of the two compounds than gave the best results with sodium nitrate alone.

The preferred composition is one part of sodium gluconate, six parts of caustic soda, and eight to ten parts of sodium nitrate. The composition is employed in a water solution, normally using from six to eight ounces per gallon of caustic soda. That is, enough of the composition is employed to give a concentration of six to eight ounces of caustic soda per gallon of solution. Thus, in a composition made up of 1 pound of sodium gluconate, 6 pounds of caustic soda, and 8 pounds of sodium nitrate, 15-20 ounces are used per gallon of solution.

The polishing bath may be employed in the cold or heated. The polishing effect becomes quite evident at 160° F. or higher, but noticeable action has been produced at room temperature.

The aluminum article is normally left in the bath for a minute or two or until a maximum polishing effect on the surface has been achieved.

A combination of sodium nitrate and sodium chlorite which gave good results was as follows:

1

5 20% NaOH  
10% sodium gluconate  
50% sodium nitrate  
20% sodium chlorite

10 This was used at the rate of 16 ounces per gallon at a temperature of 205° F. for 1½ minutes on 2 S aluminum.

15 The same mixture used with only 1% sodium gluconate was also satisfactory.

2

20 The following composition employed considerably less sodium nitrate and sodium chlorite than the preceding, but likewise gave good results:

25 2.5% sodium gluconate  
62.0% caustic soda  
25.0% sodium nitrate  
10.5% sodium chlorite

30 The composition gave good results using a concentration of 14 to 32 ounces per gallon of solution. It was used at 205° F. for 1½ minutes.

35 Good polishing results were obtained using only 16 ounces per gallon at 160° F. Some results were obtained using only 4 ounces per gallon, but the results were not up to normal commercial requirements.

3

40 A bath using 25% caustic soda, 8% sodium gluconate, and 67% sodium nitrate, employed at the rate of 16 ounces of the composition per gallon of solution gave good results at 205° F.

45 Bath No. 1 was even better.

4

45 The same bath employing 80% sodium nitrate, 15½% caustic soda, and 4½% sodium gluconate was also satisfactory.

50 When used on a series of aluminum parts, the baths continued to give a polishing action so long as there was available caustic for reaction with the metal.

55 Other oxidizing agents which of themselves would not produce a polishing action, tended to make any smut formed more adherent. While smut is undesirable, so long as it is present at all, it is better to have it adherent; so that these oxidizing agents also have a value in the process.

The following formulation gave good results when employed at 16 ounces per gallon of solution at 205° F. for 1½ minutes:

|                     |
|---------------------|
| 20% caustic soda    |
| 8% sodium gluconate |
| 8% gum arabic       |
| 44% sodium nitrate  |
| 20% sodium chlorite |

This particular bath required a temperature in excess of 150° F. to give a good polishing action.

In general with the various solutions, the time of treatment varies from 1½ to 2 minutes. If too long a time is used, gas streaking is likely to occur.

Using a reflectometer with the normal satin finish resulting from the standard caustic and nitrate etching bath as zero, the results obtained by adding gluconate were 85; and using a combination of nitrate and chlorite with added gluconate, the reading was 100.

Best results have been obtained upon 2 S aluminum. Sodium gluconate, glucono delta lactone, glucoheptonic lactone, sorbitol, and mucic acid all gave good results on this form of aluminum. 24 S, 61 S and 75 S aluminum produced fair polish.

The following baths gave good results at 16 ounces per gallon, 205° F. for 1½ minutes:

|                     |
|---------------------|
| 20% NaOH            |
| 10% sorbitol        |
| 50% sodium nitrate  |
| 20% sodium chlorite |

|                     |
|---------------------|
| 20% NaOH            |
| 10% mucic acid      |
| 50% sodium nitrate  |
| 20% sodium chlorite |

Likewise the glucono delta lactone and glucoheptonic lactone were substituted in the same formula under the same conditions with good results.

In treatments of aluminum with caustic materials where a chemical reaction with the metal occurs, a dark smut is formed. Polishing aluminum in the described baths often results in a similar condition. This smut will obscure the full luster obtained on the metallic surface. Such smut can be removed mechanically by rubbing or by acidic treatment in dilute solutions of nitric, sulfuric and chromic acids or combinations of these acids. These post polishing treatments remove the interfering substances forming the smut and permit the full luster obtained from the polishing bath to be seen.

The foregoing detailed description is given for clearness of understanding only and no unnecessary limitations should be understood therefrom as modifications will be obvious to those skilled in the art.

We claim:

1. The method of forming a reflecting surface on aluminum which comprises immersing it in a caustic soda bath including a small proportion of sodium gluconate and a large amount of a dissolved oxidizing agent.
2. The method as set forth in claim 1 in which

the temperature of the bath is at least 160° F.

3. The method as set forth in claim 1 in which the bath contains water, approximately 1 part sodium gluconate, approximately 6 parts caustic soda, and 8 to 10 parts of sodium nitrate.

4. The method as set forth in claim 1 in which the oxidizing agent is sodium chlorite.

5. An aluminum etching bath comprising water, sodium gluconate, caustic soda and an oxidizing agent.

6. An aqueous solution containing 6 to 8 ounces per gallon of caustic soda, approximately one part of sodium gluconate for 6 parts caustic soda and 8 to 10 parts of sodium nitrate for each 6 parts caustic soda.

7. An aqueous solution containing 6 to 8 ounces per gallon of caustic soda, approximately one part of sodium gluconate for 6 parts caustic soda and 8 to 10 parts of sodium chlorate for each 6 parts caustic soda.

8. The method which comprises immersing an unpolished, fabricated aluminum object for a few minutes in a bath containing 6 to 8 ounces of caustic soda per gallon of water, one part sodium gluconate for 6 parts caustic soda and 8 to 10 parts of sodium nitrate for 6 parts of caustic soda whereby a mirrored surface is produced on the aluminum object.

9. The method of treating aluminum to produce a mirror-like surface thereon which comprises immersing an aluminum surface in a caustic soda bath containing an oxidizing agent of the class consisting of sodium nitrate, sodium nitrite, sodium chlorite, sodium hypochlorite, and sodium perchlorate and a proportion of a polishing compound of the class consisting of polyhydric alcohols of the formula



where  $c$  is at least 4, salts and lactones of polyhydroxy monobasic acids having the general formula  $\text{COOH}(\text{CHOH})_c\text{CH}_2\text{OH}$  wherein  $c$  is at least 4, salts and lactones of polyhydroxy dibasic acids having the general formula



wherein  $d$  is at least 2.

10. The method of treating aluminum to produce a mirror-like surface thereon which comprises immersing an aluminum surface in a caustic soda bath containing an oxidizing agent of the class consisting of sodium nitrate, sodium nitrite, and sodium chlorate, and a proportion of a polishing compound of the class consisting of polyhydric alcohols of the formula



where  $c$  is at least 4, salts and lactones of polyhydroxy monobasic acids having the general formula  $\text{COOH}(\text{CHOH})_c\text{CH}_2\text{OH}$  wherein  $c$  is at least 4, salts and lactones of polyhydroxy dibasic acids having the general formula



wherein  $d$  is at least 2.

11. The method as set forth in claim 9 in which the oxidizing agent includes sodium chlorite.

12. The method as set forth in claim 9 in which the polishing compound is sorbitol.

13. The method as set forth in claim 9 in which the polishing compound is mucic acid.

14. The method as set forth in claim 9 in which a compound of the class of glycerine and gum arabic is included in proportion to control smut.

15. A bath for polishing aluminum comprising caustic soda containing an oxidizing agent of the class consisting of sodium nitrate, sodium nitrite, sodium chlorate, sodium hypochlorite, and sodium perchlorate and a proportion of a polishing compound of the class consisting of polyhydric alcohols of the formula



where  $a$  is at least 4, salts and lactones of polyhydroxy monobasic acids having the general formula  $\text{COOH}(\text{CHOH})_c\text{CH}_2\text{OH}$  wherein  $c$  is at least

4, salts and lactones of polyhydroxy dibasic acids having the general formula



5. wherein  $d$  is at least 2.

EUGENE R. DU FRESNE.  
JOHN R. SWIHART.

References Cited in the file of this patent

UNITED STATES PATENTS

|           |       |              |
|-----------|-------|--------------|
| Number    | Name  | Date         |
| 2,168,909 | Mason | Aug. 8, 1939 |